

## UNITED STATES PATENT OFFICE

2,416,041

## MANUFACTURE OF COATED FABRIC

Paul Rolland Austin, Wilmington, Del., assignor  
to E. I. du Pont de Nemours & Company, Wil-  
mington, Del., a corporation of Delaware

No Drawing. Application October 21, 1940,  
Serial No. 362,169

1 Claim. (Cl. 117—76)

1

This invention relates to improvements in coated products and coating processes, and more particularly to the provision of coatings upon nitro-cellulose containing articles.

Conventional sheets, films or coatings consisting essentially of nitro-cellulose, or of nitro-cellulose compositions such as pyroxylin, as is well known to the art, have pronounced flexibility and possess significant toughness, durability, and abrasion resistance. When used as coatings for fabrics, the conventional ingredients of such compositions may be so adjusted, in known manners, as to facilitate whatever degree of penetration of the base fabric, or penetrational anchorage therein, may be desired. And yet, there are a number of fundamental faults in the surface qualities of the conventional nitro-cellulose products or coatings, for which faults, and in spite of the vast amount of work that has been done in the art of coating flexible fabrics, the consuming public even up to the present time has not been provided with a wholly satisfactory solution. For instance, the nitro-cellulose coatings, per se, are subject, on aging, to brittleness, decomposition, fragility and separating from their base, as by cracking and peeling in consequence of exposure and weathering; and the tendency toward exudation to the surface, of softeners used in the said coatings, increases with rises in temperature, and has been a source of considerable difficulty in the past. In fact, for reasons such as these, it has come to pass that commercial nitrocellulose coated fabrics almost invariably are prepared with topcoats having different compositions from those of the main body of the nitrocellulose coating. Moreover, the usual topcoat not only differs from the main body of the coating in plasticizer and pigmentation, as a rule, but often consists essentially of film-forming materials other than nitrocellulose, e. g., urea-formaldehyde resins or cellulose acetate. Such topcoats may serve various valuable functions, as by improving appearance, feel, surface hardness, and immunity to crocking; but hitherto it has been difficult or impossible to attain these advantages without sacrificing other important ones. For instance, a suitably glossy surface is prone to be unduly brittle, or to have poor anchorage. Also, even with the toughest topcoats hitherto available, nitrocellulose coated fabrics have been unsatisfactory in applications where weakness or brittleness of the topcoat is not to be tolerated. Thus, glazed finishes employed in artificial patent leather characteristically are brittle, and tend to crack when repeatedly flexed, or when constrict-

2

ed in a sharp bend, as in the sewing of pleats, beading, and the like. Illustrations of such cracking and splitting often are encountered during the fabrication of handbags or shoes, for instance, along lines of stitching or at points of sharp bend. Even if fabrication is completed without such cracking or splitting, early service failure brought about thereby is very frequent. In this connection, it is to be observed, moreover, that when a topcoat is used which is more brittle than the base composition, cracking of the topcoat generally is accompanied by complete cracking through of the base composition, with resultant exposure of the fabric backing; thus rendering the material unsatisfactory for further use.

This invention therefore has as an object the minimization or elimination of the aforesaid disadvantages inherent in products or coatings consisting essentially of nitro-cellulose compositions, while at the same time preserving and utilizing the aforesaid advantageous properties thereof.

This object, as well as other important but subsidiary objects which will become apparent as the description of the invention proceeds, is accomplished according to the invention, by applying to the nitro-cellulose containing base a coating consisting essentially of one or more synthetic linear polyamides of types such as described in U. S. P. 2,071,250; 2,071,253; 2,130,523, and 2,130,948. It is to be observed, with regard to the structure of these polyamides that they contain amide groups.

35



where R is hydrogen or a monovalent hydrocarbon radical) as an integral part of the main chain of atoms in the polymer. It also may be observed that in these polyamides the average number of carbon atoms in the segments of the chain separating the amide groups is at least two. Accordingly, in this specification and the claims appended thereto, the expression, synthetic linear polyamide, is to be understood as applying to polyamides not only belonging to types described in the aforesaid patents, but also coming within the limitations pointed out in this paragraph.

I have discovered that when a layer of the said polyamides is applied over a nitro-cellulose surface, in accordance with procedures such as hereinafter set forth, the adherence is a great many times as strong as that between the same polyamide and cellulose acetate, for instance, and even will survive satisfactorily a number of hours

soaking in water. Consequently, this invention makes possible the production of articles combining the hereinabove referred to advantages of nitro-cellulose products with the outstanding surfacing qualities of the polyamides. These qualities include, among others, superlative resistance to abrasion and scuffing, and to the action of steam, grease, water and oil, fireproofness in relatively high degree, as compared with ordinary lacquers and varnishes, substantially complete freedom from tackiness even at extraordinarily high temperatures, and great strength, toughness, durability and flexibility.

The aforesaid polyamides characteristically can be formed into filaments which can be cold drawn into fibers showing molecular orientation along the fiber axis. The simple polyamides, i. e., those which may be derived from a single diamine and dicarboxylic acid or from a single amino acid, exhibit as a rule high melting points, and solubility only in toxic or corrosive solvents such as in mineral acids, formic acid, and phenols. A number of more soluble polyamides are known, however, which also have increased compatibility with plasticizers, as compared with the simple polyamides. These polyamides include those prepared from laterally substituted ingredients such as beta-methyl adipic acid, polyamides prepared from diamines and dibasic acids, one or both of which contain hetero atoms of the oxygen family in the chain of atoms joining the amide-forming groups, and interpolyamides prepared from two different diamines and two different dibasic acids, such as that prepared from a mixture of hexamethylene diammonium adipate and decamethylene diammonium sebacate. Polyamides of these types generally are more or less soluble in common organic solvents, rather than merely in phenols, mineral acids, and formic and acetic acids. They also are soluble in certain unsaturated alcohols, and certain mixtures of alcohols with chlorinated hydrocarbons.

Still another series of interpolyamides are formed by the interpolymerization of at least one diamine, at least one dibasic acid, and at least one amino acid. They possess in large degree the strength, toughness, and durability characteristics of the simple polyamides, but are characterized further by their greater pliability and compatibility with modifying agents such as plasticizers and resins, as well as by improved solubility in common nontoxic solvents, as for instance, mixtures of ethanol and water. As notably valuable illustrations of such interpolyamides may be mentioned the interpolyamides prepared by interpolymerization of hexamethylene diammonium adipate with 12-aminostearic acid and/or 6-aminocaproic acid, the interpolymers prepared by interpolymerization of hexamethylene diammonium adipate (or hexamethylene diammonium suberate and/or azelate), hexamethylene diammonium sebacate, and 6-aminocaproic acid, and the interpolymers prepared by interpolymerization of hexamethylene diammonium adipate, 9-aminostearic acid and 10-aminostearic acid. A further very valuable member of the class is that prepared by the interpolymerization of hexamethylene diammonium adipate with 6-aminocaproic acid or its amide-forming derivatives, e. g. caprolactam, since this interpolymer may be prepared from readily available ingredients, and possesses good tensile strength, flexibility, and compatibility.

The interpolyamide prepared from 6 parts of hexamethylene diammonium adipate and 4 parts

of 6-aminocaproic acid, or an amide-forming derivative thereof, such as caprolactam or 6-aminocapronitrile, is particularly valuable, since it possesses good solubility in relatively non-toxic and non-corrosive aqueous alcohol mixtures, and melts at the relatively low temperature of 165-175° C. While this temperature is sufficiently high to obviate tackiness in ordinary use, it still is low enough to permit certain important fabricating steps, such as the embossing of coated fabrics. The invention therefore will be described with particular reference to this interpolymer, although it is to be understood that the description will differ only in details, as regards the carrying out of the invention with other polyamides.

The coatings may be applied over the nitro-cellulose base in a number of ways. A convenient method consists in applying a solution of the polyamide onto the base and removing the solvent therefrom by means of evaporation. Thus, in the case of the preferred interpolyamide, a mixture of 75 parts by weight of ethanol and 25 parts by weight of water may be used as a solvent, and the solution conveniently may be applied to the base in conventional industrial coating equipment. An advantage of the solvent coating method of applying the coating is that surface gloss often may be controlled not only by varying the composition of the coating, but also by varying the method of application. For instance, when the preferred interpolymer is applied from an ethanol-water solution, a high gloss may be obtained by applying thin coats and drying at elevated temperatures, while dull finish products may be obtained by applying thicker coats and allowing them to dry more slowly.

Another convenient method for applying polyamide coatings consists in applying an emulsion or dispersion of the polyamide composition to the nitro-cellulose base and subsequently removing the vehicle by evaporation. Still another method consists in laminating a preformed sheet of polyamide composition onto the nitro-cellulose base by means of heat, pressure and, if desired, an adhesive. Another method which is particularly suitable in the case of low melting polyamide compositions consists in melt coating of the nitro-cellulose base, as by dipping, spraying, or extruding a film of molten polyamide composition directly onto the same.

It is surprising that in this procedure good anchorage at the polyamide-nitrocellulose interface readily is achieved, since frequently difficulty has been encountered in effecting good adherence between the polyamides and flat, smooth, nonfibrous surfaces.

The invention is described more specifically in the following examples, in which parts are by weight unless otherwise specified.

#### Example I

A solution of polyhexamethylene adipamide in formic acid is applied to a film consisting of nitro-cellulose containing 25% of camphor, as plasticizer. The adhesion of the residual polyamide coating to the nitrocellulose, after removal of the solvent, is excellent, even after 16 hours' soaking in water.

#### Example II

Duplication of Example I, except for the employment, in place of polyhexamethylene adipamide, of an interpolyamide prepared by the interpolymerization of a mixture of equimolecular amounts of hexamethylene diammonium adipate

and decamethylene diammonium sebacate, yields the same results in Example I, insofar as the excellence of adherence to the nitrocellulose is concerned.

*Example III*

A sand blasted steel panel is coated with a primer and then with a nitrocellulose enamel, containing in addition to nitrocellulose, iron blue pigment, plasticizer and natural resin. Over the dry nitrocellulose enamel is spread a butanol solution of the interpolyamide mentioned in Example II. The solvent is removed from this polyamide topcoating by baking the panel for one hour at 115° C. The polyamide shows good adhesion to the nitrocellulose enamel. After exposing the panel out of doors for a month in summer weather with the polyamide coating facing the south at an angle of 45° from the horizontal, the polyamide coating retains its good adhesion and shows no apparent failure.

*Example IV*

A mixture of 2.25 parts of amylnbenzenesulfonamide, 30 parts of a solvent mixture comprising 2 volumes of methanol and 1 volume of trichloroethylene, and 5.52 parts of an interpolyamide having a melt viscosity of 1419 poises at 250° C., which is prepared by the interpolymerization of a mixture of 60 parts of hexamethylene diammonium adipate and 40 parts of omega-amino-capronitrile, is heated and stirred to homogeneity under reflux at 55-60° C. for 11 hours. This solution then is applied over a pyroxylin coated fabric which consists of a 1.12-53" sateen carrying 14 oz. per linear yard of 50" width of a coating composition comprising a mixture of nitrocellulose, a plasticizer therefor, and a pigment containing carbon black. This type and weight of coating is well known to the art.

The above-described polyamide topcoating solution is applied to the nitrocellulose coated fabric in commercial fabric coating equipment, by applying the solution to coated fabric, conveying the mass under a doctor knife so arranged as to spread a thin film of the solution evenly over the nitrocellulose coated fabric, and subsequently drying the coated fabric by passing it through a drying oven. The rate of application of coating is 10 yards/min., and the temperature of the drying oven is 180° F. The drying oven is 30 feet long. Three coats are applied in this manner, and about 0.5 oz. of the polyamide topcoat (based on non-volatile ingredients) is thus applied to each linear yard of the coated fabric which is 50" in width after coating.

The product is found to have greatly improved gloss and toughness, and the anchorage of the nitrocellulose to the polyamide topcoat is good. A sample of the product withstands 7500 flexes in a Schiltknecht flexing machine, such as described in Automotive Industries 49, 1262-6; whereas a sample of the untopcoated nitrocellulose coated material fails by cracking after 2000 such flexes.

A number of sandal-type slippers having pleated vamps are prepared from the product, together with samples for comparison from the untopcoated pyroxylin coated fabric and from similar pyroxylin coated fabric carrying a commercially used topcoat comprising a urea-formaldehyde resin. Whereas there is considerable cracking and splitting of the two last-mentioned compositions, especially in areas of sharp bending, as across the pleated vamp, the polyamide topcoated pyroxylin coated fabric withstands this

fabrication perfectly. Furthermore, the polyamide topcoated material is superior in service durability, the untopcoated and the urea-formaldehyde resin topcoated materials tending to fail rapidly by cracking in those areas which are subjected to repeated flexing.

Ladies' handbags also are prepared from the product of this example. As compared with present commercial pyroxylin coated fabric, the new material is markedly superior in its resistance to cracking and splitting along lines of stitching and sharp bending. The products are of attractive appearance and feel, and are not marred, scuffed, or otherwise injured after several months of use.

*Example V*

A polyamide topcoating solution similar to that described in Example IV is applied in the same manner as described therein to a base material 20 which comprises 1.12-53" sateen coated to a weight of about 14 oz. per linear yard of 50 inch width with a pigmented composition containing 20 parts of nitrocellulose and 80 parts of a drying oil. The product has greatly improved gloss and surface hardness, and the topcoat has excellent anchorage to the base material. The topcoated product also is greatly improved in toughness, and it can be flexed repeatedly or sewed into pleats or beads without cracking; whereas the untreated base material cracks and splits badly under this treatment.

*Example VI*

Interpolyamide prepared from 60 parts of hexamethylene diammonium adipate and 40 parts of caprolactam, and having a melt viscosity of 1188 poises at 250° C. is used. A solution of 23 parts of this polymer in 77 parts of a solvent comprising a mixture of 8 volumes of ethanol and 2 volumes of water is applied as a topcoat of pyroxylin coated fabric similar to that described in Example IV. During the application, the solution is maintained at a temperature as low as 40° C., the fabric is preheated to only 60° C., and the solvent evaporates from the product at 60° C. The product has a high gloss and the topcoat is well anchored to the base. The product has better resistance to cracking and flexing than either the untopcoated material or similar material carrying a current commercial topcoat containing urea-formaldehyde resin.

*Example VII*

A solution is prepared which contains 14 parts 55 of interpolyamide similar to that described in Example IV, 5.6 parts of N-beta-hydroxyethyl-*o*-methoxybenzamide, 0.75 part of the oil-soluble resinous reaction product of formaldehyde with *p*-hydroxydiphenyl, 23.1 parts of ethanol, 8 parts 60 of methyl Cellosolve, and 7.7 parts of water. This solution is applied as a topcoat over pyroxylin coated material similar to that described in Example IV. The product has a hard, extremely glossy surface, and the topcoat is well anchored 65 to the nitrocellulose. The resistance of the product to cracking upon repeated bending is markedly improved by the presence of the topcoating.

*Example VIII*

An interpolyamide is prepared by interpolymerization of 40 parts of hexamethylene diammonium adipate, 15 parts of hexamethylene diammonium sebacate, and 45 parts of omega-amino-caproic acid. A solution then is prepared 75 which contains 65 parts of this interpolymer, 21

parts of diphenyloctadecane, and 14 parts of a condensation product of propylene glycol with castor oil, dissolved at 20% solids in a solvent mixture comprising equal volumes of chloroform and methanol. This solution is used to coat nitrocellulose coated fabric similar to that described in Example IV, two coats of the solution being applied, and the solvent being allowed to evaporate at room temperature. The polyamide topcoat is well anchored, and the product has an attractive dull satiny surface. The product is very tough and pliable and has good sewing characteristics.

In a similar manner an excellent fabric was obtained by applying to a nitrocellulose coated fabric a topcoating of interpolyamide derived from 40 parts of hexamethylene diammonium adipate, 30 parts of hexamethylene diammonium sebacate, and 30 parts of caprolactam plasticized with a mixture of 1,12-diphenyloctadecane and butyl phthalyl butyl glycolate, using as solvent a mixture of 96% ethanol and water in a 90:10 ratio by volume.

*Example IX*

An interpolyamide is prepared from 262 parts of hexamethylene diammonium adipate and 374 parts of decamethylene diammonium sebacate. A solution of this interpolymer in a mixture of methanol, chloroform, and n-butanol is applied as a topcoat over nitrocellulose coated fabric similar to that described in Example IV, allowing the solvent to evaporate at room temperature. The topcoat is clear and glossy.

*Example X*

A polyester-amide is prepared from 15 parts of hexamethylene diammonium adipate and 85 parts of an equimolar mixture of ethylene glycol and adipic acid. A solution of this polyester-amide, at 33% solids in a solvent mixture comprising 7 volumes of toluene and 3 volumes of benzene-denatured ethanol, is applied as a topcoat over the type of pyroxylin coated sheeting which is in common use as bookbinding material. The product has good anchorage and an attractive glossy appearance.

The polyamide coating may be applied to the nitrocellulose base either before or after embossing of the latter. If the application of the coating is carried out prior to embossing, the product may be embossed thereafter, with the aid of standard embossing plates or rolls. Numerous decorative effects are to be achieved, however, by applying the polyamide coating after embossing of the base. Thus, in the case of an embossed pyroxylin coated fabric, attractive color effects may be obtained by pigmenting the polyamide coating with a color or shade which is different from that in the pyroxylin base coat. If such a topcoat is applied very thin, it largely accumulates in the valleys of the grain base coat, being substantially wiped off the high spots by the action of the spreading knife. There thus will result a product wherein the high spots carry the color of the base coat, while the valleys carry the contrasting color of the topcoat.

One of the most preferred embodiments of the invention takes advantage of the fact, which already has been referred to hereinabove, that relatively thick polyamide coatings of interpolyamides soluble in alcohol-water mixtures dry dull, whereas thin coatings of identical composition give a glossy finish. Thus, if such an unpigmented polyamide topcoat, as for instance a top-

coat composition containing the preferred interpolymer dissolved in ethanol-water, is applied over an embossed base, the topcoat solution will be thicker in the valleys, thus bringing about a gloss differential, the high spots being glossy and the valleys being dull. It hitherto has been necessary to apply several successive coats of different compositions, in order to achieve such effects.

When it is desired to prepare a product of extremely high gloss, the gloss of the polyamide coating or topcoating may be improved by applying to it a final wash with a polyamide solvent, such as an alcohol or an alcohol-water mixture. Frequently it is advantageous, in order further to improve the gloss, to incorporate in such a solvent wash a small amount of a relatively high boiling solvent type material. Thus, in the case of the preferred interpolyamide, which is soluble in a 75:25 weight mixture of ethanol and water, the gloss is improved by washing coatings containing this material with a solvent mixture comprising a 50:30:20 weight mixture of ethanol: methyl Cellosolve: water. The use of this mixture, or of similar mixtures, as the actual solvent in the application of the polyamide coating, also results in an improvement in gloss and brilliance, and hence frequently is advantageous, although the presence of a relatively non-solvent such as methyl Cellosolve generally causes the solutions to gel somewhat more rapidly than otherwise, at room temperature.

Suitable polyamides, in addition to those already particularized hereinabove, include those formed by the reaction of a diamine with a substantially equimolecular amount of dibasic acid or amide-forming derivative thereof, such as an ester, halide, amide, or anhydride. There may be mentioned, furthermore, polyamides formed from polymerizable amino acids of the type, R—NH—R'—COOR, where R' is a divalent organic radical and R is a univalent organic radical or hydrogen. Interpolymers derived from mixtures of the above ingredients also are very valuable, an especially valuable subclass, typified in the foregoing examples, being those interpolymers derived by interpolymerization of an equimolecular mixture of a straight chain diamine and a straight chain dibasic acid, which mixture also contains any desired amount of a polymerizable amino acid or derivative thereof. As diamines suitable for use may be mentioned tetra-, penta-, hexa-, octa-, and decamethylene diamines, as well as substituted derivatives such as 3-methyl hexamethylene diamine, diaminoisopropanol, and aromatic diamines such as m-phenylene diamine. As suitable dibasic acids may be mentioned malonic, glutaric, adipic, pimelic, suberic, sebatic acids and their substituted derivatives, such as methyl adipic acid. Also operable are amide-forming derivatives of these acids, such as esters, halides, amide, and anhydrides. Furthermore, as polyamide-forming ingredients, either alone or in admixture with the above-mentioned diamines and dibasic acids, there may be used polymerizable amino acids such as 6-aminocaproic acid, 7-aminoheptanoic acid, 9-aminononanoic acid, 12-aminostearic acid, 17-aminoheptadecanoic acid, 8-aminocaprylic acid, and amide-forming derivatives of such acids, such as esters, halides, amides, anhydrides, and lactams.

Instead of the polyamides mentioned above, which are obtained from bifunctional polyamide-forming reactants alone, there also may be used

polyamides which are obtained by including with the polyamide-forming reactants other bifunctional reactants, such as glycols, amino alcohols and hydroxy acids. Although these products contain ester linkages, they still may be referred to as polyamides, since they contain a plurality of amide linkages in the main chain and retain many of the desirable properties of the simple polyamides.

Although in general these polyester-amides, like the simple synthetic linear polyamides, do not possess fiber- or film-forming properties unless they have an intrinsic viscosity above 0.4, where intrinsic viscosity is defined as in U. S. P. 2,130,948, coatings produced with several of the three or more component interpolyamides or interpolyester-amides will be found satisfactory for some purposes, even though the intrinsic viscosity of the particular interpolyamide be less than 0.4. Polyamides having an intrinsic viscosity between 0.6 and 2.0 are particularly suitable for use on pyroxylin undercoats over flexible fabrics.

It is generally desirable to incorporate plasticizers in the polyamide coating, since these materials tend to improve gloss, anchorage, and toughness. Suitable plasticizers are phenols, aromatic sulfonamides, certain aromatic ether-amides, and long chain aliphatic esters. Polyamide plasticizers which also are solvent-type plasticizers for nitrocellulose are of especial value in this application, since they serve to improve anchorage of the polyamide to the nitrocellulose. Such plasticizers include the aromatic sulfonamides, e. g. amylbenzenesulfonamide and toluenesulfonamide, and substituted salicylamides, e. g. N-beta-hydroxyethyl-o-methoxybenzamide.

Among other plasticizers suitable for use in the polyamide coatings and of especial value in the case of the preferred polyamide interpolymers specified in the examples, may be mentioned N-ethylamylbenzenesulfonamide; phenols such as diphenylooctadecane and octyl phenol; salicylamides; and the known softeners for the polyamides, mixed, if desired, with other materials of known softening action for the polyamides or nitrocellulose, such as castor oil or derivatives thereof, high boiling aromatic or aliphatic esters, and the like. Pigments, fillers and flattening agents also may be incorporated in the coatings.

The coating compositions also may include resinous materials, waxes and other modifying agents, whether or not compatible with the polyamides. Thus, the oil-soluble types of phenol-formaldehyde resins are of especial value in contributing gloss, luster and hardness to the composition, while finely divided incompatible resins or cellulose derivatives such as cellulose acetate, are of value as flattening agents. Diatomaceous earth and aluminum stearate can also be used as flattening agents.

The choice of solvents to be used in the solvent application of the polyamide coatings will depend upon the nature of the particular polyamide which is to be applied. Thus, formic and acetic acids are general solvents for the polyamides, while certain of the polyamide interpolymers may be dissolved in alcohols such as n-butanol, or unsaturated alcohols, or in mixtures of alcohols and chlorinated hydrocarbons, e. g., mixtures of methanol and chloroform, or in alcohol-water mixtures. In general, any liquid or mixture of liquids which is a solvent for the polyamide may be used, although where possible it is preferred, for ease of recovery, to select liquids which boil between 40° C. and 150° C.

The nitrocellulose coated fabrics which are coated according to the process of the invention are, in general, those which are known to the art. The nitrocellulose undercoating usually will contain auxiliary ingredients, e. g., plasticizers, pigments, stabilizers, or the like; and may, if desired, be modified with resins, drying oils, and so forth. The flexible sheet materials carrying the nitrocellulose coating generally will be fabrics such as cotton sheetings, sateens, and twills. Fabrics formed of materials other than cotton, however, as for instance silk, rayon, nylon, and wool, also may be used. Knitted or felted constructions also may be used.

The relative amounts of nitrocellulose-containing undercoat and of polyamide-containing topcoat may be varied as desired. In the case of the nitrocellulose-containing undercoat, however, it ordinarily is preferred to apply a weight of coating at least equal to 1.5 oz. per linear yard of 50" width, since lighter weights are generally insufficient to cover the fabric, and give products of rather poor durability. Coating weights in excess of 30 oz./50" yard are not recommended, since heavier coatings often give products that are undesirably stiff. It generally is desirable to apply a relatively thin polyamide topcoat, a coating weight of 0.1-2.0 oz./50" yard being especially satisfactory.

Another use of this invention is in coating a nitrocellulose film with polyamide for use as a photographic film base. The polyamide coating serves to reduce the fire hazard and increase the life of the film in service, e. g., in a projector.

The products of this invention possess advantages in toughness, durability, appearance, and surface characteristics which render them distinctly superior to present commercial nitrocellulose products. In particular, the fabric-nitrocellulose primer coat-polyamide topcoat products of the invention are of especial value in applications where toughness is required, such as in upholstery material and shoe upper material, especially in the case of full vamp shoes.

As many apparently widely different embodiments of this invention may be made without departing from the spirit and scope thereof, it is to be understood that I do not limit myself to the specific embodiments thereof except as defined in the appended claim.

I claim:

An article of manufacture comprising a flexible fabric carrying a nitrocellulose-containing coating, and in exterior adherence thereto, a topcoat comprising an alcohol-water soluble synthetic linear interpolyamide; the said interpolyamide being substantially identical with that obtained by the interpolymerization of 6 parts of hexamethylene diammonium adipate and 4 parts of 6-aminocaproic acid.

PAUL ROLLAND AUSTIN.

#### REFERENCES CITED

65 The following references are of record in the file of this patent:

#### UNITED STATES PATENTS

| Number    | Name            | Date          |
|-----------|-----------------|---------------|
| 2,216,735 | Carothers ----- | Oct. 8, 1940  |
| 1,951,119 | Alt -----       | Mar. 13, 1934 |
| 2,227,843 | Quenelle -----  | Jan. 7, 1941  |
| 2,071,250 | Carothers ----- | Feb. 16, 1937 |
| 1,954,750 | Hopkins -----   | Apr. 10, 1934 |
| 2,260,024 | Hall -----      | Oct. 21, 1941 |
| 2,188,332 | Carothers ----- | Jan. 30, 1940 |